

June 29, 1926.

1,590,820

F. GELSTHARP

APPARATUS FOR MAKING SHEET GLASS

Filed Oct. 7, 1924

3 Sheets-Sheet 1



INVENTOR

*Frederick Gelstharp*

*by*  
*James C. Bradley*  
*secy*

June 29, 1926.

1,590,820

F. GELSTHARP

## APPARATUS FOR MAKING SHEET GLASS

Filed Oct. 7, 1924

3 Sheets-Sheet 2

卷之三

This technical drawing illustrates a mechanical assembly, possibly a press or stamping machine, featuring a base structure with vertical columns and a central horizontal beam. Key components include:

- Left Column (Left View):** Features a vertical frame with a horizontal beam (part 2) and a base (part 1). A lever system (parts 3, 9, 10) is attached to the base. A vertical rod (part 51) is connected to a top plate (part 50) and a pulley assembly (parts 15, 16, 17).
- Central Column (Main View):** A vertical column with a horizontal beam (part 2) at the top. A vertical rod (part 51) is attached to the top of the column. A pulley assembly (parts 15, 16, 17) is mounted on the top of the column. A horizontal beam (part 19) is attached to the side of the column. A vertical rod (part 54) is attached to the side of the column.
- Right Column (Right View):** A vertical column with a horizontal beam (part 2) at the top. A vertical rod (part 51) is attached to the top of the column. A pulley assembly (parts 15, 16, 17) is mounted on the top of the column. A horizontal beam (part 19) is attached to the side of the column. A vertical rod (part 54) is attached to the side of the column.
- Base Structure:** A horizontal beam (part 2) supported by vertical legs (parts 32, 33, 34) and a central vertical support (part 31).
- Labels:** Various part numbers are labeled throughout the drawing, including 1, 2, 3, 9, 10, 11, 12, 13, 14<sup>a</sup>, 16, 17, 18, 19, 20, 21, 22, 23, 24, 25, 26, 27, 28, 29, 30, 31, 32, 33, and 34.

INVENTOR

Frederick Getchings  
by  
James C. Bradley sculptor

June 29, 1926.

1,590,820

F. GELSTHARP

APPARATUS FOR MAKING SHEET GLASS

Filed Oct. 7, 1924

3 Sheets-Sheet 3

FIG. 3.



FIG. 4.



INVENTOR

Frederick Gelstharp

Aug

James C. Bradley

Aug

## UNITED STATES PATENT OFFICE.

FREDERICK GELSTHARP, OF TARENTUM, PENNSYLVANIA, ASSIGNOR TO PITTSBURGH PLATE GLASS COMPANY, A CORPORATION OF PENNSYLVANIA.

## APPARATUS FOR MAKING SHEET GLASS.

Application filed October 7, 1924. Serial No. 742,182.

The invention relates to an apparatus for making sheet glass continuously from a tank. It has for its principal objects the provision of an improved apparatus, where-  
5 in the contact of the molten glass with the clay work at the end of the tank is reduced to a minimum, thus reducing the contamination of the glass tending to cause string and ream to a minimum; and wherein the length-  
10 ening of any bubbles in the glass incident to the rolling and sizing action is reduced, so that the visibility of such bubbles in the finished product is made as slight as possible, a round or slightly elongated bubble being  
15 much less noticeable than one which is stretched to a length several times that of the original one. Certain embodiments of the invention are illustrated in the accom-  
panying drawings wherein:

20 Figure 1 is a longitudinal vertical section through the apparatus on the line I—I of Fig. 2. Fig. 2 is a transverse section on the line II—II of Fig. 1. Fig. 3 is a horizontal section on a reduced scale on the line  
25 III—III of Fig. 1. And Figs. 5 and 6 are longitudinal vertical sections through modified embodiments of the invention.

Briefly stated the apparatus consists in  
30 means for flowing a body of glass laterally over a dam or lip or through a slot or opening in the side wall of a melting tank, a table for receiving the glass where it piles up and is spread out in a layer of much greater width than the width of the outlet slot, and a pair of sizing rolls at the forward end of the table.

This procedure involved in the use of  
35 this apparatus tends to prevent an elongation of any bubbles in the glass, which the rolling would otherwise tend to produce since the lateral spreading of the glass tends to widen the bubbles laterally and thus counteracts the tendency to lengthen them in the direction in which the surfaces of the rolls are moving, and since the surface glass carrying the bubbles stiffens, as later explained, before reaching the rolls.

40 Further, since the width of the outlet slot is only a fraction of the width of the finished sheet, the area of clay (constituting the periphery of the slot and contacting with the glass) is only a fraction of what it would be, if the width of the slot approximated that of the finished sheet. The spreading

action of the sheet may be promoted by hav- 55 ing the surface of the table slant downwardly from its longitudinal center line to its side edges, and this spreading action can also be adjusted by regulating the feed or temperature or both of molten glass to the 60 table in its relation to the speed of rotation of the sizing rolls, and by shifting the angle of the table about an axis of rotation trans-  
verse to the direction of movement of the glass sheet. An alternative means of creat- 65 ing the spread is to tilt the table down from the rolls toward the tank and providing it with a water cooled back flange to support the mass of glass which is forced to spread sideways. 70

Referring to the drawings, 1 is the outlet end of a melting tank, preferably of the well known regenerator type, having an outlet 2 below the level of the glass in the tank, and contracted by means of the gate 3, supported upon suitable means 4 for adjusting its vertical position. Back of the regulating gate is a water cooled cut off gate 5, also mounted for vertical movement upon the chains 6 and adapted to entirely cut off the supply of 80 glass in case of emergencies or in case it becomes necessary to shut down the tank for any considerable time for replacements or repairs. Back of the gate 5 is a shade 7 of clay supported by the chains 8, which may be lowered to the surface of the glass when the gate 5 is lowered, so that the glass back of the gate will not be unduly chilled by the water cooled gate during the shut down. Forward of the control gate is another water 85 cooled gate 9 or cut off supported for vertical movement by the chains 10 and designed to be employed for quick and short stops. Both water cooled gates are provided with inlet and outlet pipes so that a flow of cool- 90 ing water may be circulated through them. 95

Forward of the outlet 2 in position to receive the glass, is the table 11, which is relatively short length, as compared with its width, as will be seen by reference to Figs. 1 100 and 2. The table is preferably made hollow and with a polished surface, and is water cooled by the provision of inlet and outlet connections to provide for a continuous circulation of water therethrough. It is prefer- 105 ably pivoted at its forward end as indicated at 12, and its rear end is provided with a pair of screw jacks 13, 13, so that the angle

of the table may be adjusted to meet requirements. This table is mounted upon the truck 14, in turn carried by the track 15.

Also carried by the truck in advance of the table are the sizing rolls 15 and 16, which rolls are hollow and water cooled, by means of suitable inlet and outlet connections. The rolls are connected at their ends to the tumble shafts 17 and 18, journaled at their outer ends in the standard 19, and driven by the reducing gearing comprising the worm wheels 20 and 21 on the shafts 17 and 18 and the worms 22 and 23 on the vertical shaft 24. The vertical shaft 23 is driven from the electric motor 25 through the intermediary of a gear reduction in the casing 26, and the worm wheel and worm 27 and 28, the worm wheel being carried by the vertical shaft 24 and the worm 20 being carried by the horizontal shaft 29 leading from the gear reduction in the casing 26. The motor and reduction gearing are carried by the truck, so that when replacements or repairs are required on the front of the furnace or in any of the mechanism carried by the truck, the truck can be moved laterally to give the necessary working space and get the parts away from the heat of the tank. The movement of the truck may be conveniently secured by rotating the shaft 30 which carries a worm 31 meshing with a worm wheel 32 carried by one of the axles 33 of the truck, a handle 34 being provided for turning the shaft 30.

The width of the outlet slot is preferably only from one-sixth to one-twelfth the width of the table 11, and sizing rolls 15 and 16, so that in operation the molten glass piles up on the table back of the roll and spreads laterally to a width slightly less than the width of the table. In order to promote this spreading action, the table may be crowned, so that its upper surface slopes down slightly from its rear to its forward ends and also slopes down from its longitudinal center line to its side edges as indicated in Fig. 2. The amount of spreading also depends on the relative amount of feed and temperature through the outlet 2 as compared with the speed of withdrawal by the rolls 15 and 16, and either or both of these factors are subject to regulation. Similarly, the angle of the table affects the amount of spreading and this is adjusted by means of the screw jacks 13, 13. The matter of temperature also has an effect on the movement of the glass over the table and this may be controlled by regulating the initial temperature of the glass in the tank and by the application of heat or chilling action to the glass on the table. The glass may be chilled more or less by regulating the flow of water through the table, or it may be heated by the burners 35, 36 and 37, the burner 35 extending clear across the

width of the table, while the burner 37 extends across the width of the stream of glass flowing from the outlet 2. The burner 37 also serves to regulate the extent to which the glass flows to the rear as indicated at 70 38. Under some conditions, air may be supplied through the pipe 37 instead of gas, so that a cooling effect is produced. The burners 36 are applied only at the edges of the layer of glass upon the table and control in 75 a measure the spreading action and prevent such edges from cooling too rapidly and causing cracks in the edges of the sheet.

The spreading action on the table tends to spread laterally any bubbles in the sheet, 80 this, in connection with other factors later pointed out counteracting the tendency of the sizing rolls to elongate such bubbles so that they are rendered more noticeable in the finished product. A further advantage 85 is involved in having the outlet slot 2 of narrow width, as compared with the finished sheet, in that the area of clay over which the glass flows is reduced to a minimum, thus reducing to a minimum the contamination of the glass incident to the contact with the clay. The table 11 is referred to in the claims as "stationary" (although it is adjustable) to distinguish from the type heretofore contemplated in which an endless carrier is employed, so that the surface receiving the glass moves along with it. 90

Forward of the rolls 15 and 16 is an apron carried by the truck and with rolls 40 having sprockets at their ends driven by the chain 39. The rolls carry the glass sheet 41 continuously into the leer 42. This apron and rolls are enclosed in clay walls 43 to prevent too rapid cooling of the glass, 43 being the floor which protects the metal 105 work of the truck and 44 being a portable cover which may be removed by means of the connections 45 engaging a suitable overhead crane. The space inside the clay work and the leer may be heated by gas burners 110 projecting through the openings 46. The leer may be of any approved construction but preferably is of the roller type employing the rolls 47 for carrying the glass continuously forward while being gradually 115 annealed and cooled. The rolls 47, like the rolls 40 are provided at their ends with sprockets and are driven by a chain 48.

Figure 4 illustrates a modification in which the upper surface of the table 49 is 120 inclined downwardly from its rear to its forward end to promote the forward flow of the glass and its lateral spreading. In other respects the construction is similar to that of Fig. 1 and bears similar reference numerals. 125

In the construction of Fig. 5, a clay gate 50 is employed in connection with the single water cooled gate 51, the second water cooled gate (corresponding to the gate 9 130

of Fig. 1) being dispensed with. In this construction, the angle of inclination of the table 52 is also increased.

Fig. 6 illustrates still another modification, in which the water cooled table 53 is inclined downwardly from the rolls back toward the tank, and a flange 54 prevents the glass from flowing off the table to the rear. In other respects, the construction is similar to that of Fig. 5. This is the preferred construction.

In all the forms of the invention, the tables employed are polished so as apply a smoothing action to the lower surface of the sheet drawn thereover, so that the grinding required on such side is reduced to a minimum. Further, the traction of the rolls 15 and 16, continuously and progressively, removes the bottom chilled surface or skin, as it is formed, so that at no time is stagnant glass left upon the table, thus preventing any tendency to devitrification. The chilled skin insulates, in a large measure, the molten glass above it, the chilled outside surfaces being removed automatically as the sheet is formed. If it were not for this action, it would not be practicable to pour the glass upon a stationary table in front of the rolls and continue to form a sheet from it. The lateral flow of the glass carries the major portion of any bubbles rising to the surface, and any surface impurities, to the sides of the sheet where they are least damaging to the value of the finished product, and the glass is so cooled and hardened in its surface portions by the time they pass between the rolls that the bubbles contained therein are only slightly flattened or elongated by the sizing action. This is perhaps the most important factor in the operation tending to prevent a stretching of the bubbles. In the practice of the process, the fluid surface glass in the body behind the rolls flows to the rear and sidewise from the longitudinal center line of the glass (see arrows Fig. 3) and around its side edges to the lower surface of the glass, so that a large proportion of any bubbles or impurities, are incorporated into the lower side of the sheet formed, and closely adjacent to or at such surface. This lower surface skin is very stiff, due to the heavy chill from the table, so that the rolling action cannot stretch it (and the bubbles therein embedded), and the grinding operation which follows, is effective to eliminate most of these defects from the finished product.

What I claim is:

1. In apparatus for the manufacture of sheet glass, the combination with a tank or receptacle provided with an outlet so as to permit the discharge therethrough of molten glass under the head pressure in the tank, a stationary spreading table in posi-

tion to receive the molten glass from said outlet of a width much greater than that of said outlet, a pair of sizing rolls at the forward end of the table of a length greater than the width of said outlet, and a leir in advance of said rolls.

2. In apparatus for the manufacture of sheet glass, the combination with a tank or receptacle provided with an outlet so as to permit the discharge therethrough of molten glass under the head pressure in the tank, a stationary inclined spreading table in position to receive the molten glass from said outlet of a width much greater than that of said outlet, a pair of sizing rolls at the forward end of the table of a length greater than the width of said outlet, and a leir in advance of said rolls.

3. In apparatus for the manufacture of sheet glass, the combination with a tank or receptacle provided with an outlet so as to permit the discharge therethrough of molten glass under the head pressure in the tank, a stationary spreading table in position to receive the molten glass from said outlet of a width much greater than that of said outlet, a pair of sizing rolls at the forward end of the table of a length greater than the width of said outlet, means for cooling said table and a leir in advance of said rolls.

4. In apparatus for the manufacture of sheet glass, the combination with a tank or receptacle provided with an outlet so as to permit the discharge therethrough of molten glass under the head pressure in the tank, a stationary inclined spreading table in line with said outlet below the level thereof of a width greater than its length and very substantially greater than that of the outlet, a pair of sizing rolls at the forward end of the table, and a leir in advance of said rolls.

5. In apparatus for the manufacture of sheet glass, the combination with a tank or receptacle provided with an outlet so as to permit the discharge therethrough of molten glass under the head pressure in the tank, a stationary spreading table in position to receive the molten glass from said outlet of a width much greater than that of said outlet, a pair of sizing rolls at the forward end of the table of a length greater than the width of said outlet, means for adjusting the angle of inclination of the table with respect to the rolls to regulate the spreading action of the molten glass on the table, and a leir in advance of said rolls.

6. In apparatus for the manufacture of sheet glass, the combination with a tank or receptacle provided with an outlet so as to permit the discharge therethrough of molten glass under the head pressure in the tank, a laterally extending spreading table below the level of said outlet, in position to re-

ceive the molten glass therefrom and of a width substantially greater than that of said outlet, and a pair of sizing rolls at the forward end of the table of a length greater than the width of said outlet, the said table being downwardly inclined from its longitudinal center line to its side edges to pro-

mote the spreading of the molten glass preliminary to its entrance between said rolls.

In testimony whereof, I have hereunto 10  
subscribed my name this 23rd day of Sept., 1924.

FREDERICK GELSTHARP.